

## UNITED STATES PATENT OFFICE

2,137,282

## COPPER ALLOYS

Franz R. Hensel and Earl I. Larsen, Indianapolis, Ind., assignors to P. R. Mallory & Co., Inc., Indianapolis, Ind., a corporation of Delaware

No Drawing. Application August 12, 1938,  
Serial No. 224,498

## 1 Claim. (Cl. 75—159)

This invention relates to copper alloys.

This case is a continuation in part of our pending application S. N. 164,032, filed September 15, 1937.

5 An object of the invention is to improve the physical, chemical and electrical characteristics of such alloys.

Other objects of the invention will be apparent from the following description, taken in connection with the appended claim.

10 The present invention comprises a combination of elements, methods of manufacture, and the product thereof, brought out and exemplified in the disclosure hereinafter set forth, the scope 15 of the invention being indicated in the appended claim.

While a preferred embodiment of the invention is described herein, it is contemplated that considerable variation may be made in the method of 20 procedure and the combination of elements, without departing from the spirit of the invention.

25 The present invention relates to the improvement of alloys of copper and zirconium. According to the present invention the improved alloys are made of the following elements in substantially the following proportions:

|                                                                     | Per cent  |
|---------------------------------------------------------------------|-----------|
| Metal selected from the group consisting of iron, cobalt and nickel | 0.1 to 30 |
| 30 Zirconium                                                        | 0.05 to 5 |
| Silicon                                                             | 0.05 to 3 |
| Copper                                                              | balance   |

Where high electrical conductivities are desired, it is preferred to keep the proportion of iron group 35 metal within an upper limit of 5%.

The alloys of the present invention may also contain small proportions, or even up to several percent, of zinc, tin, calcium, lithium, magnesium, phosphorus and silver. In some cases a part of 40 the silicon may be replaced by beryllium.

The silicon combines with the iron group metal or metals to form the silicide thereof and thereby imparts age-hardening characteristics to the alloy.

45 The addition of zirconium in this type of alloy not only imparts additional age-hardening characteristics, but also produces a material of corrosion resistance, high strength at elevated temperatures and superior fatigue and impact properties.

50 The alloys can be made according to standard alloying methods. A preferred method for introducing the zirconium is to prepare a hardener alloy containing a high percentage of zirconium and then introduce a predetermined amount of 55 this alloy into a copper melt, containing the other ingredients in the desired proportions.

After the alloy has been prepared according to such methods, the material may be heat treated by first quenching the alloy in the form of a billet 60 or sand casting, or any other form, from above

700° C. and subsequently aging at a temperature below 700° C. In certain cases, we have found it also advisable to use one heat treatment only, namely, the low temperature treatment, and eliminate the quenching treatment.

If the materials are processed by rolling, extruding, drawing, forging or any other fabricating methods, we have found it desirable in many cases to quench the materials from the intermediate anneals, cold working same and applying an aging treatment afterwards. This cold working before aging hastens considerably the precipitation of the dispersed phase. In addition, a certain amount of cold work may be applied after aging in order to improve the surface finish of the wrought material.

An example of an alloy produced according to the present invention is:

|           | Per cent |
|-----------|----------|
| Zirconium | 0.70     |
| Cobalt    | 2.31     |
| Silicon   | 0.73     |
| Copper    | balance  |

After quenching this alloy from 950° C. and aging at 450° C., a Rockwell B hardness of 89 was obtained, with 45% electrical conductivity. After cold working such an alloy, a Rockwell B hardness of 95 was reached.

A nickel-containing alloy, according to the invention, is as follows:

|           | Per cent |
|-----------|----------|
| Zirconium | 1.68     |
| Nickel    | 2.26     |
| Silicon   | 0.06     |
| Copper    | balance  |

The hardness of this alloy after aging reaches 50 Rockwell B and the conductivity 43%. If cold work is applied after quenching, the maximum hardness after 60% reduction is 77 Rockwell B. The material responds to cold working after complete heat treatment and the hardness is increased from 50 Rockwell B to 76 Rockwell B.

A nickel-containing alloy showing a larger amount of silicon has a composition as follows:

|           | Per cent |
|-----------|----------|
| Zirconium | 0.80     |
| Nickel    | 1.96     |
| Silicon   | 0.70     |
| Copper    | balance  |

The maximum hardness after quenching from 950° C., and aging at 450° C., was close to 90 Rockwell B, with an electrical conductivity of 30%. Cold working again increased the ultimate hardness that could be reached with this composition.

The addition of zirconium has further beneficial effects, in so far as it raises the annealing temperature, and at the same time provides a very

fine grain structure, which is highly desirable if the material is to be worked into sheets, strips, or tubing.

The composition which has exceptional merits for condenser tubing is as follows:

|            | Per cent  |
|------------|-----------|
| Nickel     | 15 to 30  |
| Zirconium  | 0.05 to 5 |
| Silicon    | 0.05 to 3 |
| 10) Copper | balance   |

While the present invention as to its objects and advantages has been described herein as carried out, in specific embodiments, it is not desired to

be limited thereby, but it is intended to cover the invention broadly within the appended claim.

What is claimed is:

A heat-treated alloy composed of 0.05 to 5% zirconium, 0.1 to 30% of a metal or a combination of metals selected from the group consisting of iron, cobalt and nickel, 0.05 to 3% silicon, and the balance substantially all copper, characterized by high hardness and further characterized by the fact that its hardness is not permanently adversely affected by temperatures in the order of 450° C. 5

FRANZ R. HENSEL.  
EARL I. LARSEN.